

Feb. 22, 1927.

1,618,491

T. L. TALIAFERRO

METHOD OF FORMING LINERS FOR METAL CAPS FOR CONTAINERS

Filed Nov. 13, 1924

FIG. 1.



FIG. 2.



FIG. 3.



Inventor

Thomas Lucien Taliaferro

By

Stewart Mason

Attorneys

Patented Feb. 22, 1927.

1,618,491

# UNITED STATES PATENT OFFICE.

THOMAS L. TALIAFERRO, OF CHICAGO, ILLINOIS.

## METHOD OF FORMING LINERS FOR METAL CAPS FOR CONTAINERS.

Application filed November 13, 1924. Serial No. 749,664.

The invention relates to new and useful improvements in the method of making liners for metal caps for containers.

An object of the invention is to provide a method of making liners wherein the facing paper for the pulp board backing or support is secured thereto by a layer of wax attached to the pulp board, adhering to a layer of wax attached to the facing paper, and wherein said wax layers are so pressed together as to become a distinct layer, not only uniting the facing paper to the pulp board, but which latter is of a sufficient thickness to form a cushionlike member which operates to cause the liner to accommodate itself to any irregularities in the glass, and effect a tight seal.

A further object of the invention is to provide a method of making a liner, wherein in a liner of the above type is also provided with a distinct layer of wax on the face thereof adjacent the content of the container, which wax layer is not only non-porous but moisture proof.

These and other objects will in part be obvious and will in part be hereinafter more fully disclosed.

In the drawings which show diagrammatically one embodiment of the invention—

Figure 1 is a sectional view of a pulp board backing or support having a coating of wax thereon;

Fig. 2 is a sectional view of a paper facing for the pulp board support having a coating of wax on each face thereof, and

Fig. 3 shows the pulp board with its wax coating and the facing paper with its wax coatings applied thereto, preparatory to the pressing of the parts thus assembled to cause the facing paper to adhere to said pulp board.

The method of forming liners is similar to a certain extent to that disclosed in my prior Patent No. 1,476,115, granted December 4, 1923. In said prior patent, the facing paper is an oiled paper, and this is secured to the pulp board by means of a wax containing a gum. While liners made after this method are perfectly satisfactory for most purposes, there are times when it is desirable to have a liner which is non-porous and moisture proof. This is not true of the oiled paper. Furthermore, it is also desirable to have a liner wherein the assembled parts include a layer which is capable of

yielding to the irregularities in the glass so as to insure a very tight seal. The purpose of the present invention is to provide a method of forming a liner which consists of 60 pulp board, a paper facing and layers of wax, which layers of wax are preferably formed of paraffin, and in the finished article, said layers perform the double function of producing a cushion effect in the assembled parts of the liner, and also producing a non-porous, moisture proof facing to which the content of the container are exposed.

To this end, I have provided a pulp board 70 1 which is coated with hot wax so as to form a layer 2 which is of appreciable thickness. The wax will form a distinct layer by itself, which adheres to the outer face of the pulp board and will not run into the pulp board 75 and saturate it. The paper facing 3 shown in Figure 2, is provided with a layer of wax 4 on one side and a layer of wax 5 on the other side. These layers are formed, of course, of the melted wax, and this results in a distinct independent layer of wax on opposite sides of the facing paper. The facing paper constructed as described above, is then placed on the wax-coated surface of the pulp board as shown in Figure 85 3. While the wax is warm, as a result of the coating of the pulp board, or as a result of applying heat to these assembled parts, pressure is applied to the coated facing paper or the coated pulp board so as to force these 90 members toward each other. This will cause the two wax layers between the pulp board and the facing paper, which contact, to strongly adhere, and in effect, form a single layer of wax of sufficient thickness to have 95 a cushion-like effect when the liner is applied to a container. This will allow the liner to conform to any irregularities in the glass, and secure as a result, a tight seal.

Furthermore, the layer 4 of paraffin on the 100 outer face of the facing paper will likewise form a distinct layer on the surface of the paper, and this layer of wax is moisture proof and is non-porous, so that if the content of the container comes in contact with the liner, it will not work through the liner and cause the sealed package to leak.

In the carrying out of the method, the pulp board is preferably cut in a long strip, the strip being substantially of the width of the 110 diameter of the liner being formed. The paraffin paper is also cut in similar strips,

and these strips are caused to adhere to each other, after which the liners are cut from the assembled parts.

The article resulting from the method described above, is not claimed in this application, but is described and claimed in my co-pending application Serial No. 749,663, filed November 13, 1924.

It is obvious that minor changes may be made in the method of assembling the parts, the essential features consisting in the utilizing of the wax to cause the facing paper to adhere to the pulp board, and the utilizing of the wax to form a cushion effect in the completed liner, and again in the utilizing of the fact that the layers of wax are non-porous and moisture proof.

Having thus described the invention, what I claim as new and desire to secure by Letters-Patent, is—

The herein described method of forming liners for metal closures for containers comprising coating a layer of pulp board with hot wax, coating a facing paper with hot wax on both sides thereof, applying said wax coated facing paper to said wax coated face of the pulp board, and while the wax is warm, applying pressure to the pulp board and facing paper to cause the contacting faces of wax to adhere.

In testimony whereof, I affix my signature.

THOMAS L. TALIAFERRO.